



US007875802B2

(12) **United States Patent**  
**Tsotsis**

(10) **Patent No.:** **US 7,875,802 B2**  
(45) **Date of Patent:** **Jan. 25, 2011**

(54) **THERMOPLASTIC-BASED, CARBON NANOTUBE-ENHANCED, HIGH-CONDUCTIVITY LAYERED WIRE**

2008/0286560 A1 11/2008 Huang et al.  
2010/0170694 A1 7/2010 Tsotsis

(75) Inventor: **Thomas K. Tsotsis**, Orange, CA (US)

FOREIGN PATENT DOCUMENTS

(73) Assignee: **The Boeing Company**, Chicago, IL (US)

WO 2005119772 A2 12/2005  
WO 2007024206 A2 3/2007  
WO 2008076473 A2 6/2008

(\*) Notice: Subject to any disclaimer, the term of this patent is extended or adjusted under 35 U.S.C. 154(b) by 199 days.

(21) Appl. No.: **12/348,623**

(22) Filed: **Jan. 5, 2009**

(65) **Prior Publication Data**

US 2010/0170695 A1 Jul. 8, 2010

(51) **Int. Cl.**

**H01B 5/00** (2006.01)

(52) **U.S. Cl.** ..... 174/126.1; 174/126.2

(58) **Field of Classification Search** ..... 174/35 MS, 174/36, 102 R, 104, 106 R, 102 A, 116, 113 C, 174/126.1, 126.2

See application file for complete search history.

(56) **References Cited**

U.S. PATENT DOCUMENTS

6,846,985 B2 \* 1/2005 Wang et al. ..... 174/391  
6,864,418 B2 \* 3/2005 Wang et al. ..... 174/391  
6,980,865 B1 \* 12/2005 Wang et al. ..... 607/121  
6,988,925 B2 1/2006 Arthur et al.  
7,118,693 B2 10/2006 Glatkowski et al.  
7,378,040 B2 5/2008 Luo et al.  
2004/0129447 A1 \* 7/2004 Beeli et al. ..... 174/125.1

\* cited by examiner

Primary Examiner—William H Mayo, III

(74) Attorney, Agent, or Firm—Armstrong Teasdale LLP

(57) **ABSTRACT**

A conductive wire includes a thermoplastic filament having a circumference and a plurality of coating layers dispersed about the circumference of the thermoplastic filament. The coating layers include a plurality of conductive layers comprising aligned carbon nanotubes dispersed therein and at least one thermoplastic layer between each pair of conductive layers.

**20 Claims, 4 Drawing Sheets**





FIG. 1



FIG. 2



FIG. 3



FIG. 4

## 1

**THERMOPLASTIC-BASED, CARBON  
NANOTUBE-ENHANCED,  
HIGH-CONDUCTIVITY LAYERED WIRE**

STATEMENT REGARDING FEDERALLY  
SPONSORED RESEARCH & DEVELOPMENT

This invention was made with United States Government support under ATP/NIST Contract 70NANB7H7043 awarded by NIST. The United States Government has certain rights in the invention.

BACKGROUND

The field relates generally to fabrication of conductors, and more specifically to conductors that incorporate carbon nanotubes (CNTs) and the methods for fabricating such conductors.

Utilization of CNTs in conductors has been attempted. However, the incorporation of carbon nanotubes (CNTs) into polymers at high enough concentrations to achieve the desired conductivity typically increases viscosities of the compound containing the nanotubes to very high levels. The result of such a high viscosity is that the conductor fabrication process is difficult. A typical example of a high concentration is one percent, by weight, of CNTs mixed with a polymer.

Currently, there are no fully developed processes for fabricating wires based on carbon nanotubes, but co-extrusion of CNTs within thermoplastics is being contemplated, either by pre-mixing the CNTs into the thermoplastic or by coating thermoplastic particles with CNTs prior to extrusion. Application of CNTs to films has been shown, but not to wires.

Utilization of CNTs with thermosets has also been shown. However, thermosets are cross-linked and cannot be melted at an elevated temperature. Finally, previous methods for dispersion of CNTs onto films have not focused on metallic CNTs in order to maximize current-carrying capability or high conductivity.

The above mentioned proposed methods for fabricating wires that incorporate CNTs will encounter large viscosities, due to the large volume of CNTs compared to the overall volume of CNTs and the polymer into which the CNTs are dispersed. Another issue with such a method is insufficient alignment of the CNTs. Finally, the proposed methods will not produce the desired high concentration of CNTs.

BRIEF DESCRIPTION

In one aspect, a conductor wire is provided. The conductor includes a thermoplastic filament having a circumference and a plurality of coating layers dispersed about the circumference of the thermoplastic filament. The coating layers include a plurality of conductive layers comprising aligned carbon nanotubes dispersed therein and at least one thermoplastic layer between each pair of conductive layers.

In another aspect, a method for fabricating a conductive wire is provided. The method includes applying a magnetic field to a solution that includes carbon nanotubes dispersed therein, the magnetic field operating to align the carbon nanotubes, passing a thermoplastic filament through the solution, a portion of the solution adhering to the thermoplastic filament resulting in a coated filament, and washing the coated filament.

In still another aspect, a method for fabricating a conductor is provided. The method includes providing a thermoplastic filament, applying a layer of sulfonated thermoplastic to the filament, along an axial length thereof, applying a conductive

## 2

layer to the thermoplastic layer, the conductive layer including carbon nanotubes dispersed therein, and alternatively repeating sulfonated thermoplastic application step and the conductive layer application step until the conductor possesses a desired conductivity.

BRIEF DESCRIPTION OF THE DRAWINGS

FIG. 1 is a flowchart illustrating a conductor fabrication process that incorporates carbon nanotubes.

FIG. 2 is a cross-sectional diagram further illustrating a conductor 50 fabricated utilizing the process of FIG. 1.

FIG. 3 is a flow diagram illustrating application of alternating layers of thermoplastics and carbon nanotubes to fabricate the conductor illustrated in FIG. 2.

FIG. 4 is a block diagram that illustrates the individual components and processes utilized in fabricating a carbon nanotube-based conductor.

DETAILED DESCRIPTION

The described embodiments seek to overcome the limitations of the prior art by placing high volume fractions of carbon nanotubes (CNTs) onto the surface of a lightweight substrate to produce high-conductivity wires. One embodiment uses a continuous process and avoids the processing difficulties associated with dispersion of CNTs within the polymer before the structure is fabricated.

One embodiment, illustrated by the flowchart 10 of FIG. 1, includes a method for producing high-conductivity electrical wires based on layer-by-layer coating methodologies and metallic carbon nanotubes (CNTs) to introduce sufficiently high concentrations of CNTs into polymeric materials resulting in a high-conductivity conductor. The focus is on high conductivity combined with high flexibility for electrical conductors instead of focus on high stiffness, high strength, or modest increases in conductivity as were prior layer-by-layer applications.

Now referring to the flowchart 10, a thermoplastic filament, sometimes referred to herein as a substrate, is provided 12. In one embodiment, a sulfonated thermoplastic layer is applied 14 to the outer surface of the thermoplastic filament. A coating, including CNTs, is then applied 16 to the sulfonated thermoplastic layer. Several alternating layers of sulfonated thermoplastic and the coating may be applied 18 to the thermoplastic filament. The assembly is then melt-processed 20 to form CNT-enhanced, high-conductivity thermoplastic conductor. The melt-processing 20 step bonds the coating to the individual thermoplastic layers. After the melt bonding process, an outer coating, such as wire insulation, can be applied to the layered assembly.

The process illustrated by the flowchart 10 allows for high volume fractions of aligned carbon nanotubes to be applied to the surface of a thermoplastic to produce high-conductivity wires using a layer-by-layer process. Such a process avoids the necessity for having to mix nanoparticles and/or nanotubes into a matrix resin, since the combination of the two may result in a compound having an unacceptably high viscosity. Continuing, the high viscosity may make processing of the resulting compound difficult.

FIG. 2 includes a cross-sectional diagram further illustrating a conductor 50 fabricated utilizing the process of FIG. 1. As shown in the cross section of conductor 50, the thermoplastic filament 60, or substrate, has a plurality of alternating sulfonated thermoplastic layers 62 and layers 64 that include CNTs therein. The layers 62 and 64 are placed around the circumference of thermoplastic filament 60. In one specific

embodiment, the layers 64 that include the CNTs are processed to include only single-walled nanotubes. While filament 60 is illustrated as being circular in cross-section, the embodiments described herein are operable with any cross-sectional configuration for the filament.

The illustrated embodiment shown in FIG. 2 includes three thermoplastic layers 62 alternating with three CNT embedded layers 64. FIG. 3 is a flow diagram 100 the further illustrates the process for fabricating a conductor with the three alternating layers 62, 64. It should be noted that the three-layer configuration is but one example of a conductor, and that fewer or additional alternating layers could be utilized depending on, for example, expense and desired conductivity. Now referring specifically to FIG. 3, one or more uncoated filaments 102 are coated 104 with a sulfonated thermoplastic in preparation for application of the CNTs. The CNTs are applied 106, for example, by passing the thermoplastic coated filaments through a polyvinyl alcohol solution which includes the CNTs. To build up the conductor to the three-layer embodiment, the filaments 102 are alternatively coated 108, 112 with the sulfonated thermoplastic and CNTs are applied 110, 114 resulting in the conductor 50 illustrated in FIG. 2.

FIG. 4 is a block diagram 150 that illustrates the individual components utilized in fabricating a carbon nanotube-based conductor. As mentioned herein, coating methodologies are utilized to introduce sufficiently high concentrations of CNTs into polymeric materials for high-conductivity wire which are applied using a layer-by-layer coating method, as opposed to previously disclosed methods that disclose the mixing of CNTs into a resin. It is believed the currently disclosed solutions are preferable because no current solution exists for making CNT-based wires, though some methods have been proposed, as described above.

Now referring specifically to FIG. 4, fabrication of the thermoplastic filaments is described. A thermoplastic material 152 is input 154 into an extruder 156 configured to output a thin filament 158 of the thermoplastic material which is gathered, for example, onto a take up spool 160.

In a separate process, a concentrated solution 170 is created that includes, at least in one embodiment, thermoplastic material 172, a solvent 174, and carbon nanotubes (CNTs) 176. The solution 170, in at least one embodiment, is an appropriate solution of CNTs 176, solvent 174, and may include other materials such as surfactants suitable for adhering to the outer surface of thermoplastic filaments. In one embodiment, the solution 170 includes one or more chemicals that de-rope, or de-bundle, the nanotubes, thereby separating single-walled nanotubes from other nanotubes. The solution 170 is further suitable for coating thin, flexible filaments with multiple monolayers of CNTs, for example in a configuration as illustrated by FIG. 2, to achieve a desired concentration. In one embodiment, the solution 170 is a portion of the fabrication that is set up for continuous dipping, washing, and drying of individual CNT layers as they are applied to the filament.

Continuing, to fabricate the above described conductor, one or more separate creels 180 of individual thermoplastic filaments 158 are passed through a bath 184 of the above described solution 170. As the filaments 158 pass through the bath 184, a magnetic field 186 is applied to the solution 170 therein in order to align the carbon nanotubes 176. In a specific embodiment, which is illustrated, the CNTs 176 that are to be attached to the filaments 158 are the single-walled nanotubes.

The magnetic field 186 operates to provide, at least as close as possible, individual carbon nanotubes for layered attach-

ment to the filaments 158. The magnetic field 186 operates to separate the de-bundled CNTs into different types and works to extract metallic CNTs that have an "armchair" configuration, which refers to the CNT having a hexagonal crystalline carbon structure aligned along the length of the CNT. Such CNTs have the highest conductivity.

The embodiments represented in FIG. 4 all relate to a continuous line suitable for coating thin, flexible, polymeric strands (filaments 152) with a layer of the CNT solution 170 at a sufficient thickness to achieve a desired concentration or conductivity. The magnetic field 186, which may be the result of an electric field, is utilized to align the CNTs 176 in the solution 170 into the same direction as the processing represented in the Figure.

15 In one embodiment, the filaments 158 emerge from the solution 170 as coated strands 190 which are then washed and subsequently gathered onto spools 192 for post-processing. As shown in FIG. 4, the coated strands 190 may be subjected to a repeatable process. For example, to fabricate the multiple 20 conductive layers as shown in FIG. 2, the filaments 158 are passed through the solution 170 and subsequently washed as many times as needed to create the number of monolayers of CNTs to create, for example, the desired conductivity. Finally, though not shown in FIG. 4, a suitable, flexible outer 25 coating may be applied to the coated strands 190 and subsequently packaged in a fashion similar to that used for metallic wire.

The described embodiments do not rely on dispersing CNTs into a resin as described by the prior art. Instead, layers 30 of CNTs are placed about the circumference of small-diameter thermoplastic filaments as described above. One specific embodiment utilizes only high-conductivity, single-walled, metallic CNTs to maximize electrical performance. Such an embodiment relies on very pure solutions of specific CNTs 35 instead of mixtures of several types to ensure improved electrical performance. The concentrations levels of CNTs to coating are optimized for conductivity, in all embodiments, as opposed to concentrations that might be utilized with, or dispersed on, films, sheets and other substrates.

40 This written description uses examples to disclose certain embodiments, including the best mode, and also to enable any person skilled in the art to practice those embodiments, including making and using any devices or systems and performing any incorporated methods. The patentable scope is 45 defined by the claims, and may include other examples that occur to those skilled in the art. Such other examples are intended to be within the scope of the claims if they have structural elements that do not differ from the literal language of the claims, or if they include equivalent structural elements 50 with insubstantial differences from the literal languages of the claims.

What is claimed is:

1. A conductor comprising:  
a thermoplastic filament having a circumference; and  
a plurality of coating layers dispersed about the circumference of said thermoplastic filament, said coating layers comprising:  
a plurality of conductive layers comprising aligned carbon nanotubes dispersed therein; and  
at least one thermoplastic layer between each pair of said conductive layers.

2. A conductor according to claim 1 wherein said aligned carbon nanotubes comprise a plurality of conductive nano-scale material elements having a hexagonal crystalline carbon structure aligned along the length of the nanotube.

3. A conductor according to claim 1 further comprising an outer coating substantially surrounding the plurality of conductive layers along an axial length thereof.

4. A conductor according to claim 1 wherein said plurality of carbon nanotubes comprise single-walled, metallic carbon nanotubes.

5. A conductor according to claim 1 wherein said plurality of coating layers is applied to said thermoplastic filament coating material comprises a solution of said carbon nanotubes and a solvent.

6. A conductor according to claim 1 wherein said plurality of carbon nanotubes are aligned in said coating material utilizing a magnetic field before application of said coating material to said filaments, the alignment along a direction of said filaments.

7. A conductor according to claim 1 wherein said plurality of coating layers are applied to said filament by passing said filament through a bath that contains the materials of the coating layers.

8. A conductor according to claim 1 comprising a plurality of the conductive layer coated filaments.

9. A conductor according to claim 8 comprising a flexible outer coating surrounding said plurality of the conductive layer coated filaments.

10. A method for fabricating a conductive wire comprising: applying a magnetic field to a solution that includes carbon nanotubes dispersed therein, the magnetic field operating to align the carbon nanotubes; passing a thermoplastic filament through the solution, a portion of the solution adhering to the thermoplastic filament resulting in a coated filament; and washing the coated filament.

11. A method according to claim 10 further comprising repeating the passing and washing steps to apply multiple conductive layers to the thermoplastic filament.

12. A method according to claim 11 further comprising applying a coating of sulfonated thermoplastic to the filament in between each layer that includes carbon nanotubes.

13. A method according to claim 10 wherein the carbon nanotubes are single walled carbon nanotubes.

14. A method according to claim 10 further comprising applying a coating of sulfonated thermoplastic to the filament prior to passing the filament through the carbon nanotube solution.

15. A method for fabricating a conductor, said method comprising:

providing a thermoplastic filament;

applying a layer of sulfonated thermoplastic to the filament, along an axial length thereof;

applying a conductive layer to the thermoplastic layer, the conductive layer including carbon nanotubes dispersed therein; and

alternatively repeating sulfonated thermoplastic application step and the conductive layer application step until the conductor possesses a desired conductivity.

16. A method according to claim 15 further comprising applying an insulative outer coating to the conductor.

17. A method according to claim 15 further comprising packaging a plurality of the coated filaments as a single conductor.

18. A method according to claim 15 wherein applying a conductive layer to the thermoplastic layer comprises:

aligning the carbon nanotubes within a solution utilizing a magnetic field, the alignment along a length of the thermoplastic filaments; and

passing the filament through the solution such that the carbon nanotubes adhere to the filament.

19. A method according to claim 15 wherein applying a conductive layer to the thermoplastic layer comprises applying single-walled, metallic carbon nanotubes to the filament.

20. A method according to claim 15 further comprising washing the filament after each application step.

\* \* \* \* \*